

July 14, 1942.

F. F. RENWICK

2,289,384

MANUFACTURE AND USE OF FLUORESCENT LEAD SULPHATE MATERIALS.

Filed Feb. 12, 1940.



Inventor

Frank Forster Renwick

By Lynn B. Morris

Attorney

## UNITED STATES PATENT OFFICE

2,289,384

MANUFACTURE AND USE OF FLUORESCENT  
LEAD SULPHATE MATERIALSFrank Forster Renwick, Ilford, England, assignor  
to Ilford Limited, Ilford, Essex, England, a  
British companyApplication February 21, 1940, Serial No. 320,173  
In Great Britain March 31, 1939

9 Claims. (Cl. 250—81)

The invention relates to the production of materials which fluoresce under the stimulus of X-rays or gamma-rays, to the production of fluorescent screens containing such materials and to the production of photographic materials embodying such fluorescent screens and suitable for the production of X-ray and gamma-ray photographs, that is so-called "radiographs."

As is well known, X-rays and gamma-rays from radium and other radioactive materials are capable of forming latent images in silver halide emulsions and it is possible therefore to make radiographs by interposing the article to be photographed between a source of X-rays or gamma-rays and a silver halide photographic emulsion.

It is also well known that the time of exposure can be reduced by making use of an intensifying screen which contains a substance, for example calcium tungstate or zinc sulphide, which fluoresces under the influence of X-rays. When an intensifying screen is placed in contact with the photographic emulsion and the emulsion and the screen are exposed to X-rays, the fluorescent light emitted produces a latent image in the emulsion more quickly than the X-rays alone.

In order to reduce the exposure time necessary to obtain a satisfactory image, it has been proposed to combine with a sensitive emulsion on a transparent support a layer of material which fluoresces under the influence of X-rays, the layer being incorporated in or on the emulsion or embodied in the support. However, such combinations of fluorescent and light-sensitive materials have not found favour in practice largely because of the difficulty and expense involved in the preparation of known fluorescent substances which might be so employed.

It has been a growing practice in recent years in industrial radiography to employ X-rays of short wavelength generated at high kilovoltages, for example 200 to 500 k. v. or alternatively to use the gamma rays from radium or its emanation, for the radiography of thick and/or very dense objects, for example heavy metal castings.

It is found that under these conditions, neither zinc sulphide nor calcium tungstate are wholly satisfactory; zinc sulphide screens only result in the shortening of the exposure time to a small degree whilst in the case of calcium tungstate the screens have to be very heavily coated with calcium tungstate in order to obtain results of any value and even then the necessary thickness of the screens makes them very costly, reduces their flexibility and results in images of poor definition.

Moreover, when used repeatedly in contact with

photographic emulsions, the usual costly types of intensifying screens soon become damaged and unfit for further use, particularly if, as is often the case in industrial radiography, they have to be bent or moulded to the shape of the object under test. There is, therefore, a need in the field of industrial radiography for a flexible sensitive material which will give radiographs free from the blemishes due to the use of a damaged intensifying screen, which will give satisfactory results with shorter exposure times than are necessary if no intensifying screen is employed, which will give its optimum intensification with thinner layers than does calcium tungstate and which will, at the same time, not be too costly.

It has been discovered, and this forms the basis of the present invention, that crystalline lead sulphate in a state of substantial purity emits blue-violet light under the influence of X-rays or gamma-rays. With X-rays of the longer wavelengths produced at low kilovoltages (i. e. 40 to 80 k. v.) it does not fluoresce so strongly as the known fluorescent substances such as zinc sulphide and calcium tungstate; nevertheless if prepared as described below, it fluoresces strongly under the influence of X-rays particularly at high kilovoltages.

Accordingly, the present invention comprises processes for the production of lead sulphate adapted to fluoresce strongly under the stimulus of X-rays or gamma-rays, fluorescent lead sulphate produced by such processes, X-ray screens wherein the fluorescent material is substantially pure crystalline lead sulphate, and X-ray sensitive material which comprises in a single unit, one or more X-ray sensitive silver halide emulsion layers, a support for such layers and a layer of fluorescent lead sulphate.

In accordance with this invention, lead sulphate material adapted to fluoresce strongly under the stimulus of X-rays or gamma-rays may be prepared by first preparing substantially pure crystalline lead sulphate and then subjecting this to heat treatment at temperatures of the order of 700 to 1000° C. and preferably between 800 to 900° C. Conveniently the heat treatment "or firing" may be effected by heating the lead sulphate in a crucible lined with calcined calcium sulphate in a muffle furnace.

The optimum length of time for the firing treatment varies with the temperature of the treatment. Many hours are required at 700° C., about four hours at 800° C., and about 1 to 2 hours at 900—1000° C. At temperatures below

750° C. the duration of the firing treatment necessary to reach maximum activity is so great that for practical purposes temperatures below 750° C. are of little value. Firing temperatures much above 900° C., are not recommended as the product tends to sinter and requires mechanical treatment to break it down before use in the production of intensifying screens. Unduly prolonged heating after reaching the maximum activity is also detrimental to the character of the product. By giving appropriate periods of firing, products may be obtained having an intensification factor exceeding 15 and frequently as high as 25 to 30.

The firing of fluorescent materials to increase their fluorescent qualities is common practice and, as is well known, in such firing operations the fluorescent materials may be mixed with other salts as fluxes before firing. This procedure may also be adopted in the present case, if desired.

The intensification factors given above relate to the use of a single thick layer of lead sulphate (sufficiently thick to give substantially the maximum emission of light from the surface of the layer) when used as an intensifying screen placed behind and in contact with a normal type of blue-sensitive X-ray emulsion and exposed to X-rays generated at 100 k. v. They are the factors by which the exposure time would have to be increased in order to give an image of equal density were no intensifying screen used.

The intensification factor of the lead sulphate depends to some extent on the method employed for the production of the initial substantially pure crystalline lead sulphate. One convenient method by which such initial material may be prepared is as follows:

A solution of a pure lead salt (other than lead sulphate) in distilled water is added to a solution of sulphuric acid, an alkali metal sulphate or another soluble colourless sulphate in distilled water, or vice versa, in order to produce and precipitate lead sulphate by double decomposition. The initial lead salt may be a salt of an inorganic acid (and lead nitrate is preferred) or it may be a salt of an organic acid, e. g. lead acetate. The lead salt should be as pure as possible and should be free from more than the most minute traces of such metals as iron, copper, nickel, cobalt, chromium and other metals which yield coloured sulphates or the sulphates of which are unstable at low or high temperatures.

Even when the purest commercially available form of the selected lead salt is used, it is usually advantageous to purify it further. One convenient method is to precipitate a small fraction of the lead by treatment of the whole lead salt solution with a small quantity of an ammoniacal solution of an alkali metal carbonate or sulphide, filter off the precipitated lead carbonate or sulphide (which may contain impurities) and then acidify and boil the mother liquor before using it for the formation of lead sulphate.

The sulphuric acid or other sulphate used to effect the precipitation should also be free from more than the most minute traces of impurities.

After precipitation, the lead sulphate is preferably washed free from mother liquors by means of a very dilute solution of sulphuric acid, and is then dried.

The lead sulphate so obtained may be used directly to form an intensifying screen in any of the manners hereinafter set forth. Its intensification factor (as defined above) varies some-

what according to the purity of the reagents and the conditions of the precipitation, and rarely exceeds 10.

As indicated above, according to a further feature of this invention, X-ray screens are produced using substantially pure crystalline lead sulphate as the fluorescent substance. For this purpose the lead sulphate may be dispersed in any suitable binding agent, e. g. a solution of a cellulose derivative or of a colourless synthetic resin, and the resulting solution cast to form a film or coated on a paper or other support. Gelatin and other hydrophilic colloids may also be used as the vehicle but are not so satisfactory as those soluble in anhydrous solvents. A fluorescent screen thus produced may be used in the usual manner of X-ray intensifying screens; i. e. it may be placed in contact with an X-ray sensitive silver halide emulsion and the emulsion and the screen exposed to X-rays, the fluorescent light emitted by the screen producing a latent image in the emulsion more rapidly than the X-rays alone.

In the accompanying drawing similar reference numerals refer to similar parts throughout the several views:

Fig. 1 is a fragmentary, enlarged, cross-sectional view of an X-ray screen in accordance with this invention in operative relation with an X-ray sensitive element.

Fig. 2 is a fragmentary, enlarged view of an X-ray sensitive element having a lead sulphate screening layer,

Fig. 3 is a fragmentary, enlarged, cross-sectional view of a modified X-ray sensitive element having a lead sulphate screening layer,

Fig. 4 is a fragmentary, enlarged, cross-sectional view of a further modified X-ray sensitive element having a lead sulphate screening layer and a thin support,

Fig. 5 is a fragmentary, enlarged, cross-sectional view of an X-ray sensitive layer having a removable membrane containing lead sulphate.

The arrangement of Fig. 1 comprises a paper support having a layer 2 of the fluorescent lead sulphate hereof imposed thereon. It is placed in operative relation with the X-ray film element composed of a transparent support 3 having X-ray sensitive emulsion layers 4 and 4' imposed on each side thereof.

According to a further feature of this invention indicated above, substantially pure crystalline lead sulphate is used to form a fluorescent layer in a unitary X-ray sensitive material consisting of one or more emulsion layers, a support (e. g. of paper or cellulosic film) and a fluorescent layer. In such a unit the lead sulphate layer is preferably situated between the emulsion and its support or is incorporated in the support. This is illustrated in Fig. 2 wherein in a transparent support 3 bears a lead sulphate layer 2' on which is imposed silver halide layer 4.

Other arrangements are possible, but it is necessary to take into account the opacity of the lead sulphate layer both to visible light and to X-rays and gamma-rays. For example, the lead sulphate layer may be on the face of the emulsion provided the support is transparent to visible light as well as X-rays and the emulsion is exposed to rays passing through the support. Such an element is shown in Fig. 3 and comprises a transparent support 3 bearing a silver halide layer 4 on which is imposed lead sulphate layer 2'. Further, if the support is very thin and transparent to visible light and X-rays, the lead sul-

phate layer may be on the back of the support as shown in Fig. 4. It comprises a thin transparent support 3' having a silver halide emulsion layer 4' on one side and lead sulphate layer 2' on the other side. When the lead sulphate layer is coated on the face of the emulsion or on the back of the support, it may be suspended in a vehicle soluble in water or dilute alkali, for example, fish glue, or an acid resin, which would permit the ready removal of the lead sulphate layer before or during processing of the emulsion. Again, the lead sulphate layer may be of such a character that it can be stripped, in the wet or dry condition, from the assembly. A layer of lead sulphate in a vehicle such as fish glue, or in a strippable material, e. g. collodion, may in consequence be coated on to the surface of the emulsion remote from the support, and the layer may be removed before processing so that the finished radiograph can be viewed by reflected light if the support is not transparent or by transmitted light if the support is transparent. Such an element is shown in Fig. 5 and comprises a transparent base 3 having imposed thereon a silver halide layer 4 which carries a collodion membrane 5 having distributed therethrough lead sulphate.

Owing to the insolubility of lead sulphate in the usual photographic developing and fixing baths, unless it is coated on the surface and removed in the manner described above, the lead salt remains in the finished radiograph and although this is a disadvantage for some purposes, it is of no importance where the support is opaque, for example of paper, and is viewed by reflected light.

X-ray sensitive material embodying a fluorescent lead sulphate layer in accordance with the invention may be produced by dispersing the fluorescent lead sulphate in a colloid vehicle, for example a cellulose derivative, a colourless synthetic resin, a solution of gelatin or the like, coating the resulting dispersion on a support by any of the usual coating methods employed in the photographic industry, drying the product and then coating a gelatino-silver halide emulsion of the type commonly employed for radiographic purposes on the top of the lead sulphate layer to form a unitary product. When a water-permeable vehicle such as gelatin is employed for the lead salt, it is preferable to apply a protective coating, for example of collodion or other varnish, to the lead sulphate layer before applying the gelatino-silver halide emulsion in order to avoid any possibility of interaction between the emulsion and the lead salt or between the materials of processing baths and the lead salt, as lead sulphate is not completely insoluble in water.

Lead sulphate material adapted to fluoresce strongly under the stimulus of X-rays or gamma-rays possesses many advantages as the active fluorescent material in an X-ray screen. Thus it is relatively cheap (compared, for example, with calcium tungstate), only a thin layer of it is necessary with the consequential advantages that flexible X-ray screens containing it are easily producible and, since it can readily be obtained in micro crystalline form, screens containing it

as the active ingredient result in radiographs of very good definition.

I claim:

1. An X-ray screen comprising a support and a layer which fluoresces under the influence of X-rays comprising substantially pure crystalline lead sulphate obtainable by heating a substantially pure lead sulphate at a temperature of 700° C. to 1000° C. for a period of at least one hour.
2. An X-ray sensitive element for radiography which comprises an X-ray sensitive emulsion, a support for the emulsion and a screen layer containing substantially pure crystalline lead sulphate obtainable by heating a substantially pure lead sulphate at a temperature of 700° C. to 1000° C. for a period of at least one hour which will fluoresce under the stimulus of X-rays or gamma-rays and so intensify the effect of the rays on the sensitive emulsion, the whole combined to form a unitary product.
3. An X-ray sensitive element according to claim 2 wherein the lead sulphate screen layer is capable of ready removal from the assembly after the emulsion has been exposed.
4. Process for the production of lead sulphate material adapted to fluoresce strongly under the stimulus of X-rays and gamma-rays which comprises heating substantially pure crystalline lead sulphate at a temperature of 700 to 1000° C. for a period of at least about 1 hour.
5. Process for the production of lead sulphate material adapted to fluoresce strongly under the stimulus of X-rays and gamma-rays which comprises heating substantially pure crystalline lead sulphate at a temperature of 800 to 900° C.
6. Process for the production of lead sulphate material adapted to fluoresce strongly under the stimulus of X-rays and gamma-rays which comprises forming substantially pure crystalline lead sulphate by double decomposition between a solution of a pure lead salt in water and a solution in water of a compound selected from the group consisting of sulphuric acid, alkali metal sulphates and other soluble colourless sulphates, drying the product and thereafter heating it at 700 to 1000° C. for a period of at least about 1 hour.
7. X-ray fluorescent lead sulphate material consisting essentially of substantially pure crystalline lead sulphate and having an intensification factor exceeding 15 and obtainable by heating substantially pure lead sulphate at a temperature of 700 to 1000° C. for a period of at least one hour.
8. An X-ray screen comprising a support and a layer of finely divided substantially pure lead sulphate uniformly dispersed in a binding medium, said lead sulphate having been fired at a temperature from 700 to 1000° C. for a period of at least one hour.
9. An X-ray screen comprising a support and a layer of finely divided substantially pure lead sulphate uniformly dispersed in a binding medium, said lead sulphate being substantially identical with that obtainable by firing substantially pure lead sulphate at a temperature from 800 to 900° C. for a period of at least one hour.

FRANK FORSTER RENWICK.